

## UNITED STATES PATENT OFFICE

2,363,012

## COMPOUNDED MINERAL OIL

Robert J. Miller and John T. Rutherford,  
Berkeley, Calif., assignors to Standard Oil Company of California, San Francisco, Calif., a corporation of Delaware

No Drawing. Application May 6, 1942,  
Serial No. 441,964

19 Claims. (CL 252—37)

This invention relates broadly to improvements in viscous mineral oils, greases and the like, and more particularly to mineral lubricating oils which are stabilized against oxidation and rendered less corrosive to bearing-type alloys and which possess superior engine performance characteristics.

The more viscous mineral oils, used as lubricants, transformer oils and the like and in greases, vary widely in chemical composition both with respect to the main or hydrocarbon components, such as the paraffins and naphthenes, and with respect to the minor or non-hydrocarbon components, such as naturally contained naphthenic acids and sulfur compounds. Moreover, processes employed in refining such oils vary the amount and nature of the hydrocarbon and non-hydrocarbon components of the oil.

It is recognized that the chemical composition of viscous mineral oils is reflected in their properties as lubricants and the like: for example, their tendency to oxidize in the presence of oxygen and form sludge; their tendency to corrode certain bearing-type alloys, such as copper-lead and cadmium-silver alloys; and their tendency to cause discoloration of pistons and sticking of piston rings. Film strength, oiliness and pour point are also influenced by chemical composition.

A great amount of attention has been given to control of the chemical composition of viscous mineral oils in order to control the properties affecting their utility as lubricants, dielectric media and the like. Besides control from the refining end, which appertains more to the removal of undesirable constituents from the oil by physical or chemical means or their conversion by heat and/or chemical reagents into more desirable products remaining in the oil, much work has been done on the incorporation in oils of chemical agents to control their properties.

In this largely empirical science of compounded oils, that is, the science of incorporating chemical substances in oils and the like there has developed the knowledge that a considerable number of distinct but interrelated properties control the final quality of the oil. Thus mineral lubricating oils all have a tendency to oxidize in the presence of air or partial combustion products of hydrocarbons, especially at high temperatures and under high pressures. Among the disadvantages of such oxidation is the formation of sludge in the oil and of solid ad-

hesive deposits on cylinder walls and in piston ring slots. Oxidized oils also tend more readily to emulsify and are, therefore, less fit for use in contact with water; therefore less fit for use as turbine lubricants. Moreover, certain oils are either initially corrosive to the aforesaid bearing-type alloys or they become corrosive after service. Some lubricating oils tend more than others to form deposits of carbon on pistons and to cause sticking of piston rings.

In the control of these and other properties it has been proposed at various times by various workers to add to viscous mineral oils one or more additives. The total number of such proposed additives is enormous and even the broad classes of organic and organo-inorganic compounds heretofore proposed as compounding agents are numerous and cover a large portion of the field of organic and organo-inorganic compounds. It may be said that there are listed in the prior art numerous compounding agents for the improvement of lubricants with respect to any of their recognized properties, such as resistance to oxidation, corrosivity, piston discoloration and piston ring sticking.

However, many of the proposed compounding agents effect improvement with regard to one property without improving other properties and many of the compounding agents effect improvement of an oil with respect to one or more selected properties but actually have a harmful effect on other properties. This is not to say that such agents of limited utility or of mixed good and bad qualities are not useful. Many of them are highly useful and some are valuable components of the highest quality mineral oil products. However, in many cases a combination of such agents is necessary to obtain all the desired and none of the undesired effects.

This problem is well illustrated by, but by no means confined to the use of certain metal salts in lubricating oils as detergents; that is, to prevent fouling and discoloration of pistons and the sticking of piston rings. While many of the proposed metal salt detergents are highly effective in their detergent action, many of them have the drawback that they cause corrosion of bearing-type alloys. Accordingly, their utility in types of service where they are brought into contact with susceptible alloy bearings is somewhat limited. In such types of service it is necessary to combine with the metal salt detergent a corrosion inhibitor. Illustrative of metal salt detergents which promote corrosion of bearing-type alloys are the metal naphthenates,

metal soaps of fatty acids, metal phenates and metal alcoholates.

Further important factors affecting the utility of a mineral oil compounding agent are its solubility in oil, its stability at high temperatures and pressures, its stability toward oxidation and its cheapness.

It is an object achieved by the present invention to improve various properties of viscous mineral oils.

It is a further object achieved by the present invention to effect improvement of viscous mineral oils by the use of certain compounding agents without producing undesired effects.

It is a still further and particular object achieved by the present invention to stabilize petroleum lubricating oils against oxidation, to inhibit their corrosiveness toward bearing-type alloys, and to bring about an improved performance of the oil with respect to piston discoloration, piston ring slot clogging, piston ring sticking and the like, all by the use of a single class of compounding agents.

Other objects achieved by the invention will be apparent from the description and the claims.

We have discovered that certain novel petroleum nitrogen base derivatives and other like nitrogen base derivatives have very superior properties as compounding agents for viscous mineral oil compositions, especially petroleum lubricating oils.

Illustrative of the nitrogen base derivative used in accordance with the invention are the products obtained by extracting the cyclic nitrogen base derivatives present in certain petroleum oils, which are largely a mixture of alkyl substituted pyridines, reducing the extracted mixture to the corresponding alkyl substituted piperidines, and reacting the reduced mixture with an equivalent amount of carbon disulfide in the presence of an aqueous caustic alkali solution. There is thus produced an alkali metal dithiocarbamate, which may be recovered by crystallization, but other metal dithiocarbamates, such as polyvalent metal dithiocarbamates, may be produced by adding a soluble salt of the polyvalent metal to the aqueous solution of alkali metal salt, thereby precipitating the insoluble polyvalent metal salt. Salts thus produced we have found to be excellent additives or compounding agents for lubricating oils and the like.

Petroleum nitrogen bases have heretofore been proposed as compounding agents for lubricating oils, for example in Ihrig United States Patent No. 1,768,910, but better results are obtained by reducing the bases and converting the reduced bases into dithiocarbamates in accordance with this invention.

The compounding agents of our invention, even when used in small amount, effect several marked improvements in viscous mineral oils, greases, and the like, especially mineral lubricating oils. Thus they increase very substantially the resistance of mineral oil to oxidation and they inhibit corrosion of alloy bearings by mineral oils and/or other additives contained in the oil. They also result in improved engine performance of the oil; that is, they decrease the amount of ring sticking, piston discoloration and oil ring slot clogging. Moreover, the compounding agents of our invention are soluble in a wide variety of oils, such as paraffin base, naphthene base and mixed base oils, and they are stable toward heat and oxygen. They are also easily prepared from readily available materials.

The wide utility of our compounding agents is an exceedingly valuable attribute. Often in the art of compounding mineral lubricating oils with improvement agents, as hereinabove mentioned, one property, such as ring sticking, is improved, but at the expense of another property, such as corrosiveness, which is harmed. We have tested lubricants containing our compounding agents with regard to several important properties and have found that each such property is improved.

The following specific examples will serve further to illustrate the invention.

#### EXAMPLE 1

##### PREPARATION OF NITROGEN BASE DERIVATIVES

A crude cracked naphtha, as obtained in the pyrogenetic cracking of a nitrogen-containing crude petroleum oil or distillate, is extracted at ordinary temperatures with dilute aqueous sulfuric acid, of a concentration generally about 50%  $H_2SO_4$ , and water-soluble sulfates of mixed petroleum nitrogen bases are thereby formed. The petroleum nitrogen bases are recovered by neutralization with a dilute aqueous alkali metal hydroxide solution, and they are sufficiently water-insoluble to permit of stratification and decantation. In a typical case, a mixture of the crude bases thus separated from a crude cracked 100°-500° F. naphtha of California petroleum origin had a specific gravity of 0.9370, a basic dissociation constant of  $4 \times 10^{-8}$ , an average molecular weight of about 146, and an A. S. T. M. distillation boiling range between 340° and 444° F. (5% point, 394°; 90% point, 418° F.). After such recovery, the petroleum nitrogen bases are reduced to secondary amines, and such reduction may be accomplished by metallic sodium in alcoholic solution, electrolytically in dilute acid solution, or by hydrogenation under pressure in the presence of a suitable catalyst. In the latter method of reduction,  $MoS_3$  deposited on charcoal may be the catalyst, and mol ratios of hydrogen to nitrogen base between 10 to 1 and 50 to 1 may be employed, at pressures of about 200 atmospheres;  $CS_2$  or an analogous sulfur carrier should be introduced, as  $(NH_4)_2S$  is formed during the reduction and desulfurization of the catalyst may prejudice the recovery of high yields of the reduced bases. The temperature of hydrogenation should be between 475° and 650° F.; 575° F. is a good average, and the temperature should not exceed 700° F. A suitable space rate is 0.3 volume of liquid charged/hour/volume of catalyst. In a typical reduction of nitrogen bases by such a hydrogenation, 56% of the bases were reduced to secondary amines, 7% were decomposed and 37% were unreduced or unreacted upon. After reduction, whether electrolytically, by metallic sodium or by hydrogenation, the secondary amines are recovered from the reaction product mixture by adjustment of pH to approximately 8.5, in aqueous solution; unreduced nitrogen bases remain water-insoluble, while the reduced bases by reason of their higher basicity pass into water solution as salts. Excess alkali metal hydroxide is then added to liberate the reduced bases, which are sufficiently water-insoluble to permit of stratification and decantation. In the above typical case, a mixture of the petroleum nitrogen bases thus reduced (in their free form) had a specific gravity of 0.848, a basic dissociation constant of  $1 \times 10^{-3}$ , an average molecular weight of 157, and an A. S. T. M. distillation boiling range between 330 and 450° F.; they appeared as a yellow liquid,

soluble to the extent of 2.5% by weight in water at 60° F.

Subsequent to the reduction of the cracked petroleum nitrogen bases to secondary amines, the corresponding alkali metal dithiocarbamic acid salts may be prepared by reacting  $CS_2$  and aqueous alkali metal hydroxide, with the nitrogen base secondary amines, in stoichiometric proportions and at atmospheric temperature, in sufficient water to produce a 50% solution of the product: the reaction proceeds in almost quantitative yield and the desired reaction products are freely water-soluble. In the above typical case, in a sequence of steps such as that outlined, there was ultimately obtained a 50% aqueous solution of a mixture of potassium reduced cracked petroleum nitrogen base dithiocarbamates appearing as an amber liquid, specific gravity 1.11 (60° F./60° F.), with nitrogen and sulfur contents of 2.56 and 11.7% respectively.

The heavier metal derivatives of these substances may be prepared by the addition of an aqueous solution of a water-soluble salt of the desired metal to an aqueous solution of an alkali metal salt of the dithiocarbamic acid derivative. For example, a dilute aqueous zinc chloride solution, added to an aqueous solution of the sodium or potassium reduced cracked petroleum nitrogen base dithiocarbamates, prepared in accordance with the methods referred to, causes the precipitation of the water-insoluble zinc salt, and this is collected, washed thoroughly with

dissolved in an S. A. E. 30 naphthalene base oil, also in an S. A. E. 30 Pennsylvania (paraffinic) oil, in amounts ranging from 0.1 to 1.0 per cent. Samples of 50 grams each of base oil and compounded oil were taken and oxygen was bubbled through each sample, the temperature of the oil being maintained at 340° F. and all other conditions, such as oxygen pressure and rate and duration of bubbling, being maintained the same for each sample. Part of the oxygen was absorbed by the oil, the amount absorbed being determined by calculating the difference between unabsorbed oxygen and the oxygen fed to the sample of oil. The results are set forth in Tables I and II below. The various metal salts in the tables refer to the above-described metal dithiocarbamates.

Table I

| Oil                            | Cubic centimeters of oxygen absorbed after |          |           |           |           |           |           |
|--------------------------------|--------------------------------------------|----------|-----------|-----------|-----------|-----------|-----------|
|                                | 0.5 hour                                   | 1.0 hour | 1.5 hours | 1.9 hours | 2.0 hours | 2.5 hours | 3.7 hours |
| S. A. E. 30 naphthene base oil | 56                                         | 146      | 226       | —         | 286       | 325       | —         |
| Same + 0.5% of K salt          | 16                                         | 30       | 58        | —         | 96        | 128       | —         |
| Same + 1.0% of Ca salt         |                                            |          |           | 80        |           |           | 230       |
| Same + 0.5% of Zn salt         | 30                                         | 70       | —         | —         | 110       | 130       | —         |
| Same + 1.0% of Zn salt         | 42                                         | 72       | 96        | —         | 120       | 144       | —         |
| Same + 1.0% of Sn salt         |                                            |          |           | 78        |           |           | 234       |

Table II

| Oil                                                | Cubic centimeters of oxygen absorbed after— |           |          |            |           |           |            |           |
|----------------------------------------------------|---------------------------------------------|-----------|----------|------------|-----------|-----------|------------|-----------|
|                                                    | 0.5 hour                                    | 0.92 hour | 1.0 hour | 1.42 hours | 1.5 hours | 2.0 hours | 2.42 hours | 2.5 hours |
| S. A. E. 30 Pennsylvania (paraffinic) oil          | 68                                          |           | 130      | 45         | 178       | 254       |            | 302       |
| Same + 0.5% of Zn salt                             |                                             | 38        |          |            |           | 57        | 69         |           |
| Same + 0.5% of Zn salt + 0.5% metal alkyl phenate  |                                             | 66        |          |            |           |           | 90         |           |
| Same + 0.25% of Zn salt + 0.5% metal alkyl phenate |                                             | 80        |          | 94         |           | 112       | 224        |           |
| Same + 0.1% of Zn salt + 0.5% metal alkyl phenate  |                                             | 82        |          |            |           |           | 170        |           |

water, and dried. Other heavier metal derivatives suitable in the practice of our invention, for example, the lead salt, may be similarly prepared.

From the properties and reactions of the dithiocarbamates as well as those of the cracked petroleum nitrogen bases from which they are derived, it is deduced that the dithiocarbamates of this invention are predominantly one or more, probably a mixture of the substances having the following structural formulae:



In the above formulae,  $R_1$ ,  $R_2$  and  $R_3$  represent alkyl groups, which may be attached at the points shown or at other points on the piperidine ring, and  $R_1$  and the sum  $R_2+R_3$  each contains an average of 5 carbon atoms.

**EXAMPLE 2**

## OXIDATION TESTS

Potassium, calcium, zinc and tin (stannous) salts, prepared as described in Example 1, were

## CORROSION AND ENGINE TESTS

55 **Bearing metal corrosion test.**—This test is described in United States Patent No. 2,228,658 to Farrington et al. at page 3, right-hand column, lines 27 to 65. Briefly, the test comprises bubbling air through an oil maintained at 300° F. 60 and at 24 hour intervals weighing strips of copper-lead and cadmium-silver bearing-type alloys which are kept immersed in the oil, to determine the loss in weight of the strips. This loss in weight is a measure of the amount of corrosion, 65 being greater the greater the corrosion.

70 *Ring sticking, piston discoloration and oil ring slot clogging test (engine test).*—A single cylinder  $2\frac{1}{8}$  inch bore,  $2\frac{1}{2}$  inch stroke Lauson gasoline engine is operated, using compounded and uncompounded lubricating oils as lubricants, for 60 hour periods at 1600 revolutions per minute with the jacket temperature maintained at  $375^{\circ}$  F. and the sump oil temperature at  $220^{\circ}$  F. These conditions are such as to promote rapid formation of carbon and varnish on the cylinders and

pistons and sticking of the piston rings. At the end of each 60 hour run the engine is disassembled and the results noted. The piston appearance is rated as follows: A completely clean piston rates zero and a piston with completely black sides rates 800. Piston discoloration numbers (P. D. numbers) between zero and 800 indicate approximately, on a scale of 800, the proportion of blackening.

In Tables III and IV are given the results of the bearing metal corrosion tests and the engine tests for the various oils.

Table III

| Base oil  | Additives                                           | Weight loss of strip in milligrams |         |         |             |         |         |
|-----------|-----------------------------------------------------|------------------------------------|---------|---------|-------------|---------|---------|
|           |                                                     | Cu-Pb alloy                        |         |         | Cd-Ag alloy |         |         |
|           |                                                     | 24 hrs.                            | 48 hrs. | 72 hrs. | 24 hrs.     | 48 hrs. | 72 hrs. |
| Oil No. 1 | None                                                | 0.2                                | 0.7     | 1.1     | +0.1        | +0.2    | +0.4    |
| Do        | 0.5% Zn dithiocarbamate                             | 0.4                                | +0.9    | +1.5    | +0.3        | +0.7    | +1.1    |
| Oil No. 2 | 0.5% metal alkyl phenate                            | 4.5                                | 19.5    | 27.4    | 0           | 0       | 0       |
| Do        | 0.5% metal alkyl phenate + 0.25% Zn dithiocarbamate | 1.2                                | 5.3     | 24.4    | 0           | 0       | 0       |
| Do        | 0.5% metal alkyl phenate + 0.5% Zn dithiocarbamate  | 0.8                                | 1.0     | 1.9     | 0.1         | 0.1     | 0.3     |
| Oil No. 3 | None                                                | 1.6                                | 4.5     | 11.2    | 0.1         | 0.1     | 0.1     |
| Do        | 0.5% Zn dithiocarbamate                             | 0.9                                | 1.3     | 1.9     | 0.1         | 0.2     | 0.4     |
| Do        | 0.75% metal alkyl phenate                           | 18.5                               | 107.3   | 166.6   | 5.9         | 111.9   | 215.4   |
| Do        | 0.5% metal alkyl phenate + 0.25% Zn dithiocarbamate | 1.0                                | 17.2    | 51.9    | 0.1         | 8.5     | 31.9    |
| Do        | 0.5% metal alkyl phenate + 0.5% Zn dithiocarbamate  | 0.7                                | 2.6     | 16.2    | 0.1         | 0.2     | 0.3     |
| Oil No. 4 | None                                                | 0.2                                | 0.0     | +0.6    | +0.2        | +0.2    | +0.6    |
| Do        | 1% Zn dithiocarbamate                               | 0.0                                | 0.0     | +2.2    | +0.1        | +0.1    | 0.0     |
| Do        | 0.5% metal alkyl phenate                            | 17.0                               | 44.0    | 81.5    | 3.7         | 36.5    | 56.7    |
| Do        | 0.5% metal alkyl phenate + 0.5% Zn dithiocarbamate  | 0.7                                | 7.6     | 34.7    | 0.1         | 0.4     | 0.1     |

Table IV

| Base oil  | Additives                                          | No. of rings stuck | PD No. | Per cent ring slot clogging | Cu-Pb bearing weight loss in milligrams |
|-----------|----------------------------------------------------|--------------------|--------|-----------------------------|-----------------------------------------|
| Oil No. 1 | None                                               | Two                | 600    | 80                          | 16                                      |
| Do        | 0.5% Zn dithiocarbamate                            | None               | 250    | 70                          | 8                                       |
| Oil No. 2 | 0.5% Zn dithiocarbamate + 0.5% metal alkyl phenate | do                 | 255    | 0                           | 3                                       |

In Table III, a plus sign (+) in front of a number indicates that the alloy strip increased rather than decreased in weight. In Tables III and IV the base oils designated as Oil No. 1, Oil No. 2, etc. were the following types of oil:

Oil No. 1—Naphthene base.

Oil No. 2—California paraffin base.

Oil No. 3—Pennsylvania paraffin base.

Oil No. 4—Gulf Coast naphthene-paraffin base.

With reference to Table III, a loss in weight of either alloy strip of 15 milligrams in 72 hours represents about the borderline between a non-corrosive and a corrosive oil. Oils which sustained more than 15 milligrams loss of weight in 72 hours under the conditions of the bearing metal corrosion test are classifiable as "corrosive" oils, whereas oils which sustained less loss of weight are classifiable as "non-corrosive" oils. Further with respect to Table III, it will be noted that the zinc dithiocarbamate in no case rendered corrosive a normally non-corrosive oil, and in those cases where an oil was corrosive, the zinc dithiocarbamate greatly decreased the corrosiveness of the oil or rendered the oil non-corrosive.

Besides the petroleum nitrogen base derivatives hereinabove described, other similar nitrogen base derivatives, whether of petroleum origin or not, and whether the nitrogen base is of natural or synthetic origin, may be advantageous used in lubricating oils, and such use is within the purview of the invention.

Thus piperidine derivatives of the dithiocar-

bamate type; that is, in which the ring nitrogen of the piperidine residue is also the nitrogen of the characteristic dithiocarbamate group



may be used whatever the source of the piperidine or piperidine homologue. Also, other rings may replace the piperidine ring; for example, four, five and seven member rings. Typical examples of nitrogen base derivatives coming within

the broader aspects of the invention are the following:



Four membered ring



Five membered ring



Six membered ring



Seven membered ring

In these formulae the nitrogen rings may be substituted, as by alkyl groups, and M stands for the hydrogen equivalent of a metal; that is, so much of a metal as is not satisfied by other groups. Part or all of the valencies of a polyvalent metal may be satisfied by the nitrogen ring dithiocarbamate radical.

Broadly speaking, therefore, the present invention comprises the use in oils and the like of ni-

trogen ring dithiocarbamates represented by the following formula:



in which M is the hydrogen equivalent of a metal, X is a nitrogen-containing ring attached to the



group through the ring nitrogen, and C and S have their usual significance.

Preferably, however, we use those nitrogen ring dithiocarbamates in which, as in the herein described reduced petroleum nitrogen base dithiocarbamates, the nitrogen ring bears one or more alkyl substituents, and preferably those that contain at least 5 carbon atoms in the alkyl group or groups attached to the nitrogen ring. The most advantageous oil compounding agents of all the petroleum nitrogen base dithiocarbamates described hereinabove in detail.

Various metals may take the place of M in the above type formula; for example, sodium, potassium, copper, magnesium, calcium, strontium, barium, zinc, aluminum, tin, lead, chromium, molybdenum, manganese, iron, cobalt and nickel, although zinc and calcium are preferred.

Some oils, such as certain excessively treated oils, are normally corrosive to certain bearing alloys. Other oils are normally non-corrosive toward such alloys but are rendered corrosive thereto by the addition of various compounding agents, such as the aforementioned metal salts of organic acids or acid-acting substances, comprising certain metal naphthenates, metal soaps of fatty acids, metal phenates and metal alcoholates. Specifically, the following metal salts of organic acids, phenols and alcohols, among others, cause oils to be corrosive or more corrosive toward bearing-type alloys: aluminum naphthenate, calcium naphthenate, magnesium naphthenate, aluminum stearate, calcium stearate, calcium phenylstearate, calcium dichlorostearate, calcium benzolstearate, aluminum oleate, calcium oleate, barium cetylphenate, calcium cetylphenate, potassium cetylphenate, calcium octadecenolate, sodium octadecenolate. Many of these compounding agents are useful in lubricating oil, for example for their detergent effect. Combinations of such agents with the metal dithiocarbamates of the present invention are very useful. The combined detergent effect and/or other useful properties of the corrosive metal salt and the corrosion inhibiting effect and other useful properties of the dithiocarbamate are thereby obtained.

The preferred compounding agent of our invention is the aforesaid zinc dithiocarbamate of Example 2 prepared by reacting reduced petroleum nitrogen bases with  $\text{CS}_2$  in the presence of caustic alkali solution, and precipitating the zinc salt by adding a soluble zinc salt to the alkali solution, as described in Example 1. The preferred combination of agents according to our invention are mixtures of our metal dithiocarbamates and metal alkyl phenates, in particular the said zinc dithiocarbamate and alkaline earth metal alkyl phenates such as calcium cetyl phenate and other alkaline earth metal phenates containing higher alkyl substituents. These mixtures combine in high degree the valuable properties of each component with fewer if any of the disadvantages of the components taken separately.

Quite small amounts, on the order of 0.05 to 4 per cent by weight based on the finished product, of the dithiocarbamates of the invention are in most cases sufficient to bring about the desired effect in viscous mineral oil compositions, although in special cases greater amounts may be advisable. Greater amounts, for example from 5 to 50 per cent by weight on the oil, may also be incorporated in mineral oil to produce a concentrate, which can be more conveniently stored and transported and, when required, mixed with more oil to produce lubricant containing the proper proportion of compounding agent. The dithiocarbamate may be combined with another additive, such as one of the aforementioned metal salt detergents, in such a concentrate.

The compounding agents of our invention are useful generally in combination with mineral oils, as in crankcase oils, gear lubricants, transformer and switch oils, greases, etc.

The dithiocarbamates disclosed hereinabove are claimed as components of greases in our co-pending application Serial No. 521,438, filed February 7, 1944.

25 We claim:

1. A composition of matter comprising a viscous mineral oil and a small amount, sufficient to stabilize the oil against oxidation of a nitrogen base derivative in which the nitrogen forms part of a ring and is attached to the group



wherein M is the hydrogen equivalent of a polyvalent metal.

35 2. The composition of claim 1, wherein the metal M is an alkaline earth metal.

3. The composition of claim 1, wherein the metal M is zinc.

40 4. A compound lubricating oil, comprising a major amount of viscous petroleum oil and a minor amount, sufficient to improve substantially the lubricating characteristics of the oil, of a nitrogen based derivative in which the nitrogen forms part of an alkyl substituted ring, the total number of carbon atoms in the alkyl substituent or substituents being at least 5, and in which the nitrogen is attached to the group



50 wherein M is the hydrogen equivalent of a polyvalent metal.

5. The oil of claim 4, wherein the nitrogen base is an alkyl substituted piperidine.

6. The oil of claim 4, wherein the metal M is an alkaline earth metal.

7. The oil of claim 4, wherein the metal M is zinc.

60 8. A compounded mineral lubricating oil, comprising a major amount of a petroleum oil of lubricating viscosity and a minor amount, sufficient to improve substantially the lubricating characteristics of the petroleum oil, of a polyvalent metal dithiocarbamate of which the dithiocarbamate nitrogen atom forms part of a ring derived from nitrogen-containing cracked naphtha by extraction of pyridine bases from the naphtha, reduction of the extracted pyridine bases, and reaction of the reduced pyridine bases with carbon disulfide.

65 9. The compounded oil of claim 8, wherein the petroleum lubricating oil is a naphthenic oil.

10. The compounded oil of claim 8, wherein 70 the petroleum lubricating oil is a paraffinic oil.

11. The compounded oil of claim 8, wherein the metal salt is an alkaline earth metal salt.

12. The compounded oil of claim 8, wherein the metal salt is a calcium salt.

13. The compounded oil of claim 8, wherein the metal salt is a zinc salt.

14. A compounded lubricating oil, comprising a major amount of petroleum oil of lubricating viscosity, a metal salt selected from the group consisting of metal salts of organic acids, metal salts of phenols and metal salts of alcohols, said metal salt being present in the oil in small amount sufficient to improve piston cleanliness, inhibit piston ring sticking and promote corrosion of alloy bearings, and a small amount, sufficient to inhibit corrosion of alloy bearings, of a nitrogen base derivative in which the nitrogen forms part of an alkyl substituted ring, the total number of carbon atoms in the alkyl substituent or substituents being at least 5, and in which the nitrogen is attached to the group



wherein M is the hydrogen equivalent of a poly- 25

15. The oil of claim 14, wherein the corrosive metal salt is a metal naphthenate.

16. The oil of claim 14, wherein the corrosive metal salt is a metal soap of a fatty acid.

17. A composition of matter, comprising a concentrated solution in viscous mineral oil of a nitrogen base derivative in which the nitrogen forms part of a ring and is attached to the group

10



wherein M is the hydrogen equivalent of a polyvalent metal.

15

18. A compounded lubricating oil comprising a petroleum lubricating oil and about 0.1 to 4 per cent by weight based on finished oil of a polyvalent metal dithiocarbamate in which the dithiocarbamate nitrogen forms part of an alkylated piperidine ring.

19. The oil of claim 18, wherein said polyvalent metal salt is a zinc salt.

ROBERT J. MILLER.  
JOHN T. RUTHERFORD.